

# UNITED STATES PATENT OFFICE.

LARRY L. COMEAU, OF HAVERHILL, MASSACHUSETTS.

## ENAMELED-LEATHER SOFTENER AND PROCESS OF MAKING THE SAME.

1,049,674.

Specification of Letters Patent.

Patented Jan. 7, 1913.

No Drawing.

Application filed February 10, 1910. Serial No. 543,126.

*To all whom it may concern:*

Be it known that I, LARRY L. COMEAU, of Haverhill, in the county of Essex and State of Massachusetts, have invented an Improvement in Enameled-Leather Softeners and Processes of Making the Same, of which the following is a specification.

This invention relates to certain improvements in compositions of matter which are primarily designed to soften enameled or "patent leather," so that the enamel will not crack when the leather is bent or strained when used, in the manufacture of shoes thereby obviating factory damages and greatly increasing the wearing qualities of the shoes. I accomplish this object by preparing a composition of matter which is adapted to be applied to both the enameled side and the flesh side of the leather and to be worked into the same thoroughly, and which preferably consists of a mixture of neat's-foot oil, soap, alcohol, kerosene and water. In order that these substances may be properly combined for my purpose the mixture thereof is performed by a certain process.

According to my process I first provide two separate mixtures which consist respectively of a solution of hard soap, water and neat's-foot oil in the proportion of  $\frac{1}{4}$  pound of soap to two quarts of water, and  $\frac{1}{2}$  pint of neat's-foot oil; and a mixture consisting of one pint of grain alcohol, one pint of water,  $\frac{1}{2}$  pint neat's-foot oil, and one pint of kerosene. These two mixtures are then united and thoroughly intermingled so that the resulting mixture consists of: 1 pint neat's-foot oil, 1 pint alcohol, 1 pint kerosene,  $2\frac{1}{2}$  quarts of water, and  $\frac{1}{2}$  pound of soap. The resulting mixture is a liquid, but, if it is desired in the form of a paste, the proportion of soap is increased.

While approximately the proportions, above specified, are desirable, they are not essential, as they may be varied within reasonable limits without seriously impairing the efficaciousness of the mixture, for example, the alcohol, though desirable, is not essential.

This mixture, when applied to the enamel of the leather, will cause it to become flexi-

ble and pliable, so that cracking will be prevented, and this is accomplished without injury to the enamel or in any way detracting from its luster. Enameled leather is liable to become sticky in warm temperatures, but all liability of such an occurrence is avoided by applying my composition to the enamel.

As in the manufacture of enameled leathers nearly all of the oils in the leather are removed, the leather loses much of its pliability and becomes brittle, so that it is made less durable; but, after being treated with the composition above described, its original characteristics are, to a large extent, restored.

The principal advantage to be derived from the use of my composition is in connection with the lasting operation of shoes, in which it has been customary to moisten the vamp before applying the same to the last, so that it will be more pliable. This also permits the leather to be stretched, as it is drawn into place and secured. When the leather dries, it shrinks again, and frequently cracks or splits. When, however, the leather is treated with my composition previous to lasting, it is not only made sufficiently pliable and flexible, to enable the lasting operation to be satisfactorily performed, but the condition in which it is placed is retained, so that it will not tend to shrink while on the last in the remaining portion of the process of manufacture.

I claim:

1. The herein-described process of making a leather softener, which consists in first preparing a mixture of neat's-foot oil and dissolved soap, and a mixture of neat's-foot oil, alcohol, and kerosene, and then uniting the two mixtures into a common mixture.

2. The herein-described composition of matter, or leather softener, which consists of a mixture of neat's-foot oil, soap, and kerosene, substantially in the proportions set forth.

3. The herein-described composition of matter, or leather softener, which consists of a mixture of neat's-foot oil, alcohol, soap, and kerosene, substantially in the proportions set forth.

4. The herein-described composition of matter, or leather softener, which consists of a mixture of neat's-foot oil, alcohol, soap, kerosene and water, substantially in the proportions set forth.

5. The herein-described composition of matter, or leather softener, which consists of a mixture of approximately one pint neat's-foot oil, one pint alcohol, one pint

kerosene, two and one-half quarts of water, 10 and  $\frac{1}{4}$  pound of soap.

In testimony whereof, I have signed my name to this specification, in the presence of two subscribing witnesses.

**LARRY L. COMEAU.**

Witnesses:

**L. H. HARRIMAN,**  
**H. B. DAVIS.**